

Jan. 27, 1959

R. J. GOLDBERG ET AL  
REDUCTION OF DYE ABSORPTION IN HARDENED  
GELATIN RELIEF MATRICES  
Filed Oct. 8, 1957

2,870,704



Fig. 1



Fig. 3



Fig. 2

Inventor  
Richard J. Goldberg  
Earl M. Olds, Jr.  
by Robert Lushman & Shover  
Attest

# United States Patent Office

2,870,704

Patented Jan. 27, 1959

1

2,870,704

## REDUCTION OF DYE ABSORPTION IN HARD-ENED GELATIN RELIEF MATRICES

Richard J. Goldberg, North Hollywood, and Earl M. Olds, Jr., Van Nuys, Calif., assignors to Technicolor Corporation, Hollywood, Calif., a corporation of Maine

Application October 8, 1957, Serial No. 688,921

6 Claims. (Cl. 101—149.1)

One well-known method of making photographs is to make a relief image in gelatin of the scene. The relief can be formed, for example, by exposing a silver containing gelatin layer through a transparent support, developing the image adjacent the support with a developer which hardens the gelatin coextensively with the developed silver, and etching or dissolving the unhardened surface gelatin with warm water. The relief thus formed is called a matrix and can be stained with dye which is then transferred by imbibition to another gelatin layer to form a print. If a relief matrix is made for each color aspect of a scene, suitably dyed, and successively transferred in superposition to the print, a reproduction of the scene is made in full color.

Relief matrices are normally made so that the resulting gelatin relief absorbs more dye than needed to transfer the color aspect of the scene to be reproduced. This is corrected by subjecting the saturated relief to a controlled water wash to remove the dye in excess of the amount desired. This operation is called "washback" and apparatus suitable for this purpose is disclosed in U. S. Patent No. 2,602,387.

Occasionally relief matrices are produced which absorb more excess dye than this subsequent washback operation can correct, especially where such matrices exceed the design limits of machines designed for the purpose. Additionally, some matrices, initially satisfactory, become too absorbent on repeated reuse in making a series of imbibition prints. Such overly-absorbent or overscale relief matrices have heretofore been discarded.

The principal object of this invention is to provide a method of reducing the dye absorption, without destroying the contrast, of a hardened gelatin relief matrix which absorbs dye in excess of the amount which can be corrected by the washback step in the transfer process.

In accordance with this invention, the method comprises the steps of treating an overscale matrix with a proteolytic enzyme bath for a predetermined time sufficient to solubilize only a portion of the gelatin and dissolving this portion with a solvent, preferably warm water. By this method the dye absorption is reduced by the desired amount without destroying the contrast of the relief. Preferably the enzyme bath has a temperature of about 70° to 80° F., a pH between about 4 and 11, and the warm water has a temperature of about 120° to 140° F. The amount of excess absorbency of a matrix, and hence the extent of the enzyme treatment required, is determined in conventional manner, for example by making density measurements of a print made from the matrix and comparing with density standards of the scene.

A specific embodiment of this invention is illustrated in the accompanying drawing in which

Fig. 1 is a flow chart;

Fig. 2 is a plot of the density characteristic curve of a magenta matrix before and after treatment; and

Fig. 3 is a plot showing the relation between the time of enzyme treatment in a standard enzyme bath and the reduction in matrix washback required.

2

Referring to Fig. 1, overscale and overly-absorbent relief matrices are restored to the proper range or degree of dye absorbency by treatment with a proteolytic enzyme bath A for a time sufficient to solubilize enough gelatin 5 to reduce the matrix absorbency to a predetermined amount, etching B with warm water to dissolve the solubilized gelatin, and drying C the etched relief. By this method the dye absorption of an overly-absorbent matrix is reduced to the desired range without destroying the contrast of the relief. The preservation of contrast is illustrated by the density curves shown in Fig. 2, curve 1 being the curve of a magenta matrix before treatment while curve 2 is the characteristic of the same matrix after treatment.

10 The amount of gelatin hydrolyzed and removed from the matrix and the resulting reduction in dye absorption is dependent on the concentration and temperature of the enzyme solution and on the time of treatment. The catalytic activity of each enzyme is usually at a maximum at a temperature not greatly above room temperature. An increase in temperature brings about an increase in the rate of reaction but also causes a loss in enzyme 15 action. At temperatures above 120° F. loss in enzyme action becomes very rapid. Enzyme activity is lowered as the temperature is lowered below room temperature. Thus the preferred solution temperature is 75° F.  $\pm 5^\circ$ . The pH of enzyme solutions is usually around 7.0 but is generally not critical between the limits of about 4 and 11. Beyond these limits there is a rapid loss in 20 activity. At a fixed temperature, solution activity is directly proportional to enzyme concentration and activity. While other activities could be used, solutions having enzyme activity equivalent to about .002 gram of pure 25 crystalline trypsin per liter of water have been found suitable for the present invention.

30 The amount of excess absorbency and hence the length of enzyme treatment required is determined by conventional means. One method is to make a density standard of the scene or scenes as they are photographed and to 35 compare the density of a print made from the matrix with this standard. These density differences are correlated with the time in seconds of immersion of the matrix in a given enzyme bath necessary to bring the density measurements into satisfactory agreement, that is, into such agreement that the final adjustments can be 40 made in the washback step in the transfer process.

45 Conveniently in the usual transfer process, the density differences are first correlated with the seconds of treatment in a given washback apparatus and then the seconds of immersion in a given enzyme bath are correlated with the reduction in required washback thereby obtained. Then when more washback is required than the apparatus 50 can provide, the requirement is reduced by treatment for the correlated time in a standardized enzyme bath. Fig. 55 3 illustrates the reduction in required washback in seconds with various immersion times in an enzyme solution containing 4.5 grams "Amprozyme 200" (activity equivalent to .002 g./l. pure crystalline trypsin) per liter in water at  $75^\circ \pm 5^\circ$ , curve 3 representing yellow and magenta matrices and curve 4 representing cyan dyed 60 matrices.

65 While it is more convenient and hence preferred to vary the time of immersion in a solution of fixed activity to correct matrices of varying amounts of over-absorbency, the same result can be achieved by using a standard time and varying the concentration of enzyme or by a combination of both.

70 The enzymes useful for this invention are proteolytic enzymes or any mixture of enzymes containing a proteolytic enzyme. Examples are trypsin, Amprozyme 200, Rhozyme PF, Rhozyme P11, Protozyme P concentrate,

## 3

Protozyme S, and Gelatinase. ("Amprozyme" and "Protozyme" are trademarks of Jacque Wolfe and Co., "Rhozyme" is a trademark of Rohm and Haas Co., and Gelatinase is a product of Takamine Laboratory, Inc.) The action of the enzyme is to enhance the hydrolysis of the protein structure by catalytic action, the hydrolyzed gelatin then being dissolved with warm water. This catalytic action of the enzyme proceeds without regard to the presence or absence of metallic silver in the gelatin.

Many of the commercial enzymes, particularly those which are mixtures of enzymes, have activities which vary from sample to sample. The proper concentration can be selected by comparison with the desired concentration of pure trypsin which has a substantially constant activity or by preparing a solution with the new sample and then increasing or decreasing the enzyme concentration to bring it into agreement with a desired curve as illustrated in Fig. 3. The method presently used comprises measuring the density loss of a standard test film with a densitometer; for example the Erpi densitometer, in a bath of a desired activity for a standard immersion time, for example 100 seconds. For reproducible results, this then becomes the standard for comparison. On a new batch of enzyme, test solutions of various concentrations are made and the density losses on the same test film are plotted against concentration to determine the concentration which gives the desired loss at the same conditions. Each new solution made is tested to assure that it gives the desired loss, water or enzyme being added if necessary.

The enzyme treated relief matrix is fed into a warm water bath, preferably a cascade, to remove the retained enzyme solution and the hydrolyzed gelatin. The preferred temperature for this etch is 130° F.  $\pm$  10°. At 150° F. the unhydrolyzed gelatin will begin to dissolve while at 90° F. the solution time is unduly long. On removal from this etching or water bath, the relief is given a rinse in water at the same temperature and the relief is then dried, either by allowing evaporation at room temperature or by forced drying. While the water rinse has been found desirable to avoid streaking, it can be omitted, especially where solution make-up water is allowed to contact the emerging film. The matrix can then be dyed and used in a conventional manner. By this method over-scale matrices can be reclaimed and used rather than discarded as heretofore.

This invention may be better understood by reference to the following specific examples:

## EXAMPLE NO. 1

A matrix representing the yellow aspect of a scene was tested and found to be over-scale by about 12 seconds more washback treatment than could be provided by the washback step in the transfer process. This matrix was treated as follows:

- (1) Bathe for two minutes at 75° F. in a water solution (pH 7.0) containing .002 gram per liter of pure crystalline trypsin,
- (2) Etch in water at 130° F. for one minute, and
- (3) Dry.

By this treatment the absorbency of the matrix was substantially reduced, without adversely affecting its contrast, to an amount readily corrected in the conventional washback step.

## EXAMPLE NO. 2

The same matrix referred to in Example 1 was treated as follows:

- (1) Bathe for two minutes at 75° F. in a water solution (pH 7.0) containing 4.5 grams per liter "Amprozyme No. 200," an enzyme mixture of bacterial origin sold by Jacque Wolfe & Co.,
- (2) Etch in water at 130° F. for one minute, and
- (3) Dry.

## 4

## EXAMPLE NO. 3

A second matrix representing the cyan aspect of a scene was tested and found to be over-scale by about 16 seconds. This matrix was treated as follows:

- (1) Bathe by immersion for 97 seconds at 75° F. in a water solution (pH 7.0) containing .002 gram per liter trypsin,
- (2) Etch in water at 130° F. for one minute,
- (3) Water rinse at 130° F., and
- (4) Dry.

## EXAMPLE NO. 4

The matrix of Example 3 was treated as follows:

- (1) Bathe by immersion for 97 seconds at 75° F. in a water solution (pH 7.0) containing 1.0 gram per liter of "Rhozyme PF," an enzyme sold by Rohm and Hass Co.,

(2) Etch in water at 130° F. for one minute,

(3) Rinse in water at 130° F., and

(4) Dry.

Any convenient backing can be used such as glass, Celluloid, plastics, etc. In each of the examples given, the gelatin was supported on acetate film. The process also operates irrespective of the dyes used. However conventional magenta, yellow and cyan dyes used to dye gelatin reliefs should be employed. Examples of such dyes are as follows:

## Yellow

|    |                                                            |       |       |
|----|------------------------------------------------------------|-------|-------|
| 30 | Chlorazol Brilliant Yellow 3G (ICI), C. I. Direct Yellow 4 | grams | 2.00  |
|    | Chlorazol Fast Orange ER (ICI), C. I. Direct Orange 37     | do    | 0.25  |
|    | Acetic acid, glacial                                       | mls   | 10.00 |
| 35 | Water to make 1.00 liter                                   |       |       |

## Magenta

|    |                                                         |       |       |
|----|---------------------------------------------------------|-------|-------|
| 40 | Chlorazol Fast Pink BK (ICI), C. I. Direct Red 75       | grams | 3.60  |
|    | Durazol Red 2B (ICI), C. I. Direct Red 81               | do    | 0.45  |
|    | Amanil Brilliant Violet R (AAP), C. I. Direct Violet 30 | do    | 0.50  |
|    | Acetic acid, glacial                                    | mls   | 50.00 |
| 45 | Water to make 1.00 liter                                |       |       |

## Cyan

|    |                                               |       |       |
|----|-----------------------------------------------|-------|-------|
| 50 | Disulphine Green B (ICI), C. I. Acid Green 9  | grams | 0.25  |
|    | Solway Celestol B (ICI), C. I. Acid Blue 27   | do    | 1.25  |
|    | Lissamine Green BN (ICI), C. I. Acid Green 50 | do    | 0.40  |
|    | Acetic acid, glacial                          | mls   | 30.00 |
| 55 | Water to make 1.00 liter                      |       |       |

<sup>1</sup> "Color Index," second edition 1956, The American Society of Textile Chemists and Colourists.

It should be understood that this disclosure is for the purpose of illustration only and that this invention includes all equivalents and modifications falling within the scope of the appended claims.

We claim:

1. For reducing the dye absorption of a hardened gelatin relief matrix which absorbs dye in excess of the amount necessary correctly to reproduce a color aspect of a scene, the method which comprises treating the matrix with a proteolytic enzyme bath for a predetermined time sufficient to solubilize only a portion of the gelatin and dissolving said gelatin portion with a solvent, thereby reducing the dye absorption without destroying the contrast.

2. For reducing the dye absorption of a hardened gelatin relief matrix which absorbs dye in excess of the amount necessary correctly to reproduce a color aspect of a scene, the method which comprises treating the ma-

trix with a proteolytic enzyme bath for a predetermined time sufficient to solubilize only a portion of the gelatin and dissolving said gelatin portion in warm water, thereby reducing the dye absorption without destroying the contrast.

3. Method according to claim 2, wherein the enzyme bath has a temperature of approximately 75° F.

4. Method according to claim 2, wherein the warm water bath has a temperature of approximately 130° F.

5. Method according to claim 2, wherein the enzyme bath has a pH between about 4 and 11.

6. The method of reducing the dye absorption without

destroying the contrast of a hardened gelatin relief matrix which absorbs dye in excess of the amount necessary to correctly reproduce a color aspect of a scene, comprising the steps of determining by density measurements the amount of excess absorbency of a matrix, treating said matrix in a proteolytic enzyme bath for a time sufficient to solubilize that portion of the gelatin necessary to eliminate the excess absorbency beyond that normally corrected by washback, and dissolving said portion in warm water.

No references cited.